

April 20, 1937.

G. F. McMAHON

2,077,429

CIRCUIT INTERRUPTER AND ARC EXTINGUISHING LIQUID THEREFOR

Original Filed March 2, 1933



Inventor:  
George F. Mc Mahon

By *Moore Jackson Bottles & Drums*

Serial No. 2,077,429

## UNITED STATES PATENT OFFICE

2,077,426

## CIRCUIT INTERRUPTER AND ARC EXTINGUISHING LIQUID THEREFOR

George F. McMahon, Chicago, Ill., assignor to  
Schweitzer & Conrad, Inc., Chicago, Ill., a corporation of DelawareApplication March 2, 1933, Serial No. 659,266  
Renewed September 25, 1935

45 Claims. (Cl. 200—120)

My invention relates primarily to circuit interrupters of the type wherein cessation of current flow is brought about by the successive steps of first forming an arc, i. e., a flow of current through a conductive vapor or gas; second, the deionization of the arc to render it insufficiently conductive to maintain current flow; and, third, interposing in the previous path of the current flow a nonconductor or insulator of sufficient dielectric strength to prevent reestablishment of the current flow.

The apparatus in which I preferably embody the present invention is liquid filled fuses of the well known S & C. type. Also, the invention may be employed in liquid filled circuit breakers of known or preferred type.

Whereas the invention is primarily concerned with the extinguishing of arcs, it is not intended to limit the dielectrics herein disclosed to such use only. These dielectric liquids may be employed as fluid insulators in such apparatus as depends for its operativeness upon the integrity of the insulation. Examples of this class are high tension terminals for transformers, circuit breakers, and the like, high tension cables, transformers, regulators, etc. In these devices the possibility of rupture of the insulation is never absent. Such rupture is invariably accompanied by the formation of an arc and, unless the dielectric is substantially noncombustible, grave consequential damage may result from the secondary energy released by combustion of the dielectric.

The noncombustible dielectric arc extinguishing liquids of my present invention are valuable for both the above mentioned uses, because they have the tendency of deionize the arc and extinguish the same, thereby terminating the further release of electrical energy in addition to preventing any release of secondary energy of combustion.

In general, the possibilities of employing dielectric mediums having the two valuable properties above referred to are known. See Schweitzer & Conrad patent, Reissue No. 14,879; see Ringwald Patent No. 1,862,317, and see my Patent No. 1,966,901, issued July 17, 1934. The said disclosures relate to the provision of a suitable liquid or solid dielectric for the same class of service as the dielectric mediums herein disclosed, and the liquids and solids herein disclosed may be employed in structures such as are disclosed in the aforesaid patents and application.

In the development of fuses employing dielectric liquids and/or solids of the present class, the

practical difficulties of securing a uniformly dependable product are very great. Whereas certain compounds, considered by themselves, might appear highly desirable for the present service when they are put to the test by employing them in contact with the necessary operating parts, under practical conditions of manufacture and use, they are found to be quite unsuitable.

Among the chief difficulties encountered in the manufacture and use of liquid and/or solid filled fuses of the S & C. type are the following:

1. Impurities contained in the commercially available compound employed in making up the dielectric.

2. Impurities introduced into the dielectric or the container in the course of manufacture. Such impurities may come from the glass sleeve, the brass and copper parts, or from the surrounding atmosphere, e. g., moisture, oxygen, etc. These impurities may react with a correctly selected dielectric and develop highly detrimental action, such as corrosion of the metal parts.

3. The heat developed by the fuse standing under electric load, or received from the surrounding medium, or atmospheric changes of temperature which may run to extremes in either direction. Heat generally tends to accelerate such chemical action as occurs in devices of the present type.

4. Chemical activity may be caused or induced by light, particularly where certain impurities are present. Chemical action, due to impurities, may continue as a progressive action, and even if it occurs at a slow rate will, in course of time, develop serious defects in the fuse.

5. If any active impurities are present they may, under the influence of current flow, enter into an electrolytic action which tends to continue so long as the device carries current.

6. Upon blowing of the fuse a highly complex action occurs. First, the fuse element becomes heated to incandescence and melts, and an arc is formed. There is therefore a sudden release of electrical energy at high temperature. This fusing of the link is a desirable step in two ways; first, in the preferred form of fuse it releases mechanically the terminal so that it may be retracted by the spring; second, it substitutes a metal vapor for a solid conductor. The tendency under such release of heat at high temperature is for the dielectric to be broken down, and new compounds formed. This action should not be exothermic, because it would merely release more energy when there is already an excess of energy released in the arc. Also, if

should not release combustible liquids, vapors, or gases, because upon venting to the atmosphere this would result in increasing the energy released, in addition to increasing the danger to adjacent structures and the personnel.

The second chief action which it is desired to realize is that of deionizing the arc. The arc extinguishing material here has a complex action, which consists essentially in reducing the conductivity of the ionized gases and vapors. Probably this action is physical as well as chemical and electrical. The desired result is cessation of current flow and the interposition between the terminals of a dielectric of such strength that the arc is unable to restrike or reestablish itself. If the fuse vents to atmosphere, it is desirable that the ejected material should not be inflammable, noxious, or corrosive.

Electrical devices of the class to which this invention relates, such as fuses, circuit breakers, transformers, etc., are often required to stand in exposed situations and under load for long periods of time. Particularly fuses of the type herein referred to, which have a glass container, permit the entry of light to the dielectric liquid. They are thus subjected to adverse influences over long periods. During such periods, heat due to current flow or to atmospheric conditions and actinic effects, chiefly from sunlight, are applied to the liquid. Hence, any tendency for the liquid dielectric to undergo a chemical change has ample opportunity to act.

The first object of the present invention is to provide a circuit interrupter of the self-contained or enclosed type employing an arc extinguishing medium which is acted upon by the arc to facilitate circuit interruption.

A further object of the present invention is to provide an improved fuse device of the enclosed or substantially enclosed type employing an arc extinguishing medium which gives the device as a whole improved characteristics.

A further object is to improve the methods of manufacture of fuses and like devices, and particularly the method of preparing and utilizing the arc extinguishing dielectric.

A further object is to improve the stability of the dielectric and of the entire device in which it is utilized.

50 A further object is to improve the reliability of devices employing liquid dielectrics of this class and to extend the useful life of the same.

A further object is to provide an improved form of liquid filled fuse having dependable certainty of operation over extended periods of time.

A further object is to provide an improved fuse of the type above recited.

Other objects will appear from the following specification, drawing, and claims.

In the accomplishment of the above and other objects I employ as the preferred embodiment of my invention a liquid filled fuse of the S. & C. type in which the arc extinguishing liquid is a halogen derivative of a hydrocarbon found to be suitable for its primary service of arc deionization and having the necessary physical characteristics of boiling point, freezing point, density, etc.

A liquid or series of liquids suitable from the above standpoint is disclosed in my aforesaid Patent No. 1,966,901. The liquid or class of liquids therein disclosed, even in the pure state, is free of injurious reaction with water which may be contained in the fuse casing, even though exposed to sunlight. However, if air is present,

the oxygen thereof, either alone or in combination with moisture, and particularly in the presence of sunlight, reacts with the liquid to break it down and induce chemical changes which result in release of reagents which attack the metal parts of the fuse causing deterioration of the same.

In the development of fuses of this class, it has been found desirable to provide a definite expansion chamber to receive and condense vapors and gases evolved upon blowing of the fuse, such condensation being sufficient to prevent venting of the fuse casing to atmosphere upon operation of the fuse except on severe overloads. This expansion chamber may be filled with a neutral gas, but preferably is merely air filled. When so air filled the oxygen content of the fuse tends to react with the arc extinguishing dielectric, even though impurities have been removed so far as feasible. When impurities are present they will generally accelerate the breakdown of the dielectric.

Now, according to one phase of the present invention, I introduce into the dielectric a small amount of a so-called preservative. This is preferably aniline. It may be any suitable derivative of aniline, such as aniline dyes. I intend to include in this class compounds which are nitrogen containing derivatives of aromatic hydrocarbons and also aliphatic hydrocarbons. Other materials may be employed. The material must not interfere with the original arc extinguishing and dielectric properties of the filling liquid. It should not be used in large quantities, neither should it cause deterioration by its combination with the impurities or the products of decomposition of the filling liquid. In other words, neither the material itself nor its products of combination should interfere with the properties or functions of the filling liquid. The aforesaid and like material may be employed not only in the fuse itself, but as a medium for purifying such liquids as tetrachloroethylene and the like, in the commercial process of manufacture or preparation for some particular use. A small amount of aniline, or the like, may be allowed to remain in the liquid, i.e., tetrachloroethylene, or the like, as a preservative.

Now, in order to acquaint those skilled in the art with the manner of constructing and practicing my invention, I shall describe in conjunction with the accompanying drawing a typical embodiment of one phase of my invention, and then describe the manner of practicing the various phases of my invention.

In the drawing the single figure is a longitudinal vertical section through a fuse device embodying my invention.

In the drawing I have shown a fuse of the S. & C. type, which type is well known in the market. The fuse comprises a glass sleeve 1, which forms the main part of the housing for the working parts. A closed sleeve or cap 2 is cemented upon the lower end of the sleeve 1 to form a tight joint and seal. The sleeve 2 forms the lower extremity electric terminal for the device. At the upper end of the glass sleeve 1 a metallic ferrule 3 is similarly cemented. The ferrule 3 has an extension forming an enlarged chamber 4, and this chamber may be provided internally with cooling fins 5, preferably formed in the shape of thin annular sheet metal rings or a helical coil of thin strip stock for the purpose of affording a large superficial cooling and condensing surface for the

vapors and gasses discharged into the chamber 4 upon operation of the fuse device. They may be integral with the walls of chamber 4. Also, if desired, cooling fins 11, preferably disposed vertically to promote natural circulation, may be secured upon the outside.

The upper end of the chamber 4 is closed off by a releasable vent cap 6 which may cover the entire cross section of the chamber 4, or may be limited to a smaller area. The cap 6 is preferably cemented in place by a suitable cementitious material giving a bond of known strength for the purpose of releasing the internal pressure at a value which will be below that dangerous to the integrity of the fuse housing as a whole. Within the chamber 4 a suitable buffer 7 formed by a pair of crossed rods or a stamped spider or casting may be employed to intercept discharge of the movable terminal upon violent blowing of the fuse. This buffer may be yieldably supported on the coiled strip 5. A tubular chamber or passageway 8 within which the arc or a part of the same is adapted to be confined is provided in the upper part of the fuse housing. This tubular chamber 25 or passageway is defined by a sleeve 9, which is made of insulation such as fiber or successive layers of a suitable impregnated sheet, such as paper or the like. The sleeve 9 is supported at its upper end in a transverse head or barrier plate 10, which is externally threaded and cooperates with threads formed internally within the ferrule 3. The threads indicated at 12 preferably have a predetermined strength against rupture by pressure within the glass sleeve 4, so that if excessive pressure is generated within the glass sleeve 4, the head or barrier plate 10 may be driven outwardly to provide greater relief to the internal pressure. The buffer 1 may also be expelled in case of too great internal pressure beneath it.

This barrier plate or head 10 is preferably formed of insulating material, although it may be made of metal, if desired. Its chief function is mechanical. It may be made of a phenolic condensation product, bakelized fiber, or of other insulating material, suitable for the purpose to which it is devoted. It may be imperforate outside the central opening or may have restricted openings to release some of the pressure outside the arcing chamber 8.

The sleeve 9, defining the tubular chamber 8, is secured at its upper end in an opening in the head or barrier plate 10. This may be merely a press fit. The intention is to have a certain definite holding force for holding the sleeve 9 in the head 10, which holding force will be overcome when the pressure within the glass sleeve rises to predetermined value. The theory of the construction is to retain as much pressure within the sleeve 4 as it is safe to carry, and progressively releasing the same if it tends to rise above predetermined limits, by first expelling the sleeve 9 and then the head 10.

The tubular chamber or passageway may be designated as an arcing chamber in the present device, for the reason that the fusible link is disposed therein, or immediately adjacent the upper end thereof, and upon fusing of the fusible link 13, the pressure so generated and the heat incidental to fusion and the consequent arc does not strike the glass sleeve 4, but is confined within the insulating sleeve 9.

The fusible link 13 is preferably a silver wire fastened electrically and mechanically to a short cylindrical terminal 14 at its upper end, and

fastened to a metallic rodlike terminal 15 at its lower end. The upper terminal 14 has a threaded slot extending through a hole centrally disposed in the connecting member 16. A nut 17 clamps the terminal member 14 to the connecting member 16. The connecting member 16 is preferably a cup-shaped piece of sheet copper or brass with the shallow rim thereof slotted, so as to provide spring fingers engaging radially within the bore 18 and bearing endwise against a shoulder 19 formed substantially at the juncture of the head 18 and the sleeve 3.

The terminal 14 and the terminal 15 are provided with connecting means for coupling to the ends of a conductor 20 of high resistance, but great mechanical strength. This conductor, termed in the trade the strain wire, is preferably a piece of high tensile strength alloy steel, such as a nickel-chromium-iron compound. Preferably this strain wire 20 has loops formed at its opposite ends, these loops extending into bores in the terminals 14 and 15, and transverse pins 22 and 23 mounted in the terminals extending through the loops of the wire 20, so as to give a loose pin and linkage connection, having the effect of universal joints of limited freedom. The fuse wire 13 is preferably a silver wire, the central part of which is coiled about the strain wire 20, and the ends are straight, extending axially into slots of longitudinally extending openings in the terminals 14 and 15, the metal of such slots or openings being battered or riveted over the surface of the fuse wire to make good electrical and mechanical connection.

The lower terminal 15 carries a liquid director 24, as by means of a series of radially projecting pins 25. The upper end of the terminal 15 projects into the explosion chamber 8, and the upper end of the liquid director 24 extends into the lower end of sleeve 9. The terminal 15 is connected by shunting conductor 26, which is in the form of a stranded flexible cable, to the lower external terminal 2. A coil spring 27 stressed in tension is connected between the lower external terminal 2 and the terminal 15. The coiling of the spring 27 is to pull the terminal 15 with its connected liquid director 24 downwardly. The interior of the fuse housing is filled up to the liquid level line indicated at A with a suitable liquid which will be described more in detail later. This level is approximately  $\frac{1}{4}$  in. below the top of the lower fuse terminal 15 at room temperature i.e., 25°C. The height of the sleeve 9 may be varied considerably, depending upon the specific mode of operation desired on the part of the fusible link, but in general it has been found to be quite satisfactory to have the liquid disposed below the body of the fusible link, so that heating of said link is not influenced to any great extent by the presence of the liquid, and vice versa. The upper part of the housing above the liquid level is preferably filled with air, although I contemplate, within the present invention, the substitution of inert atmosphere, for example, nitrogen, argon, or any gas which is neutral toward the filling liquid and is not too soluble therein. The liquid director 24, upon blowing of the fuse, is drawn downwardly through the body of the liquid, and while it is not fitted tightly within the sleeve 4, it acts, nevertheless, like a piston in a cylinder and liquid is driven through the central annular opening, and about the lower terminal 15. Inasmuch as the greatest freedom of escape from below the fused or barrier plate 10 is through the tube

lar passageway or chamber 8, the liquid so projected is discharged into the chamber 8 and is acted upon by the arc which tends to vaporize it. The liquid and vapor flows at great rapidity, in fact with violence through the said chamber or passageway 8, within which a corresponding length of the arc is confined. This violent flow of the arc extinguishing liquid and the fluids resulting therefrom, which are gas and vapor, in passing through the chamber 8 tend to deionize by condensing upon the charged particles and combining chemically with the metallic vapors and to blow the metallic vapors which were formed by melting of the fuse and strain wires, endwise into the chamber 4.

The connecting plate 16 is preferably provided with a series of openings, which allows gases and vapors to flow therethrough towards the chamber 4, but if the pressures are sufficient, this connecting plate 16, and the upper terminal 14 carried thereby, may be driven into the chamber 4.

The continued downward movement of the terminal 15 tends to submerge it in the liquid contained within the housing, and such movement extends the length of the arc, and also brings more of the arc extinguishing liquid within the influence of the arc with further flow of the gaseous medium, that is, vapors and gases, out through the passageway 8, tending to deionize the arc both by condensation upon the charged particles and by the constant substitution of a non-ionized dielectric medium, and an outward sweep of the ionized gases and vapors.

If the blow is so violent as to require expulsion of the sleeve 9, it may be driven upwardly into the chamber 4; likewise, the head or barrier plate 10 may be expelled. In the event that the condensing and cooling capacity of the chamber 4 and its cooling means, is not sufficient to keep down the pressure below that for which the cap 6 is adjusted, this cap may be blown off to vent the chamber 4 and connected parts to atmosphere.

For usual conditions of protection, the blowing is not so violent as to require release of the vent cap 6.

The arc extinguishing dielectric, which is employed in the present fuse, is preferably composed chiefly of a halogen substitution product of a hydrocarbon.

As explained in my copending application, Serial No. 503,481, trichloroethylene ( $C_2HCl_3$ ) and tetrachloroethylene ( $C_2Cl_4$ ) in suitable proportions may be employed to advantage in devices of this character. Furthermore, solid dielectrics of the same general class, such, for example, as hexachloroethane ( $C_2Cl_6$ ) may be dissolved in one or the other of the aforesaid liquids, or in a mixture of both. The mixture of trichloroethylene and tetrachloroethylene is generally free from decomposition by sunlight in the presence of moisture, but both tetrachloroethylene and trichloroethylene are easily oxidized under the action of light when they are allowed to be in contact with atmospheric air at ordinary atmospheric temperatures. Tetrachloroethylene is decomposed in sunlight in the presence of oxygen into phosgene ( $COCl_2$ ) and trichloroacetyl chloride ( $CCl_3COCl$  or  $C_2Cl_4O$ ). Trichloroacetyl chloride is easily oxidized further by water to form trichloroacetic acid ( $C_2HCl_3O_2$ ) and free hydrochloric acid. This hydrochloric acid of course tends to attack the metal parts of the fuse or the metallic structure with which it is in contact. In the present construction, the ferrules 1 and 2 of the fuse are

made of brass, which is readily attacked by chlorine. The terminals 14 and 15 are also made of brass, and the spring and shunting cable 27 and 26, respectively, and their connected parts, are all made of brass or copper. While the fuse element is preferably made of silver, and is less subject to attack, nevertheless the formation of hydrochloric acid within the interior of the fuse housing, which is highly undesirable, tends to cause deterioration of the fuse element and to result in possible change of rating, and also to contaminate the arc extinguishing liquid itself.

Trichloroethylene is also easily oxidized in the sunlight in the presence of oxygen. While in the preferred embodiment of the invention, the fuse housing is hermetically sealed, the upper part of the housing is preferably filled with atmospheric air. Also a certain amount of oxygen tends to enter in the course of manufacture through absorption by the surfaces of the various materials entering into the construction of the device.

The decomposition of trichloroethylene results chiefly in carbon dioxide, hydrochloric acid and phosgene. While there may be various intermediate products in the decomposition of trichloroethylene and tetrachloroethylene, the final products are acid in character, corrosive to the metal parts of the fuse.

As previously explained in my copending application, the mixture of these two liquids in approximately the ratio of ninety-four parts of tetrachloroethylene and six parts of trichloroethylene gives a dielectric arc extinguishing medium which has the advantage of a low freezing point, high dielectric strength, relatively high boiling point, and excellent arc extinguishing properties. Hexachloroethane ( $C_2Cl_6$ ) may be added up to about 25% of the mixture of trichloroethylene and tetrachloroethylene. The percent of halogen content (chlorine) in the resulting liquid will be of the order of 80% to 85%, although it may be of the order of 75% to 95%, depending upon the halogen compound used.

To the arc extinguishing liquid consisting of one or more of the above halogen derivatives of a hydrocarbon I add a small amount, for example, less than  $\frac{1}{10}$  of 1% by weight of aniline as a preservative.

Aniline is basic in character. It reacts with acid substances readily, forming stable neutral compounds which do not readily corrode metals so long as aniline is present in the liquid. It tends to combine with any of the impurities which are contained within the arc extinguishing liquid, or liquids such as tetrachloroethylene, trichloroethylene, and the like, and it may serve as a preservative of these liquids for general purposes, such as fire extinguisher service, for use in electrical apparatus such as transformers, liquid filled bushings, cables, and the like.

I believe it is broadly new to employ aniline or any of its derivatives as a preservative of tetrachloroethylene or trichloroethylene, or any of the halogen derivatives of hydrocarbons such as are employed for fire extinguisher service, or the other uses to which I have referred. Also, aniline, or its derivatives, serve as an excellent purifier in the manufacture of chlorine derivatives of hydrocarbons or other halogen derivatives of hydrocarbons. Instead of using aniline, any one of its derivatives which react readily with oxygen or chlorine, or the other halogens or acid impurities which it is desired to remove, may be employed instead. Many of the derivatives of aniline, in-

cluding commercial coal tar dyes, may be employed instead of the aniline itself.

In the process of purification of trichloroethylene or tetrachloroethylene or the like, I add a suitable amount of aniline or its derivatives. The amount employed is preferably in excess of that necessary to combine with the impurities of the liquid to be treated. The liquids are thoroughly stirred and allowed to stand for a time to allow contact between the aniline and the impurities to the necessary extent. Aniline reacting with hydrochloric acid, which is a common impurity in chlorinated hydrocarbons, forms aniline hydrochloride. Reacting with trichloroacetic acid it forms trichloroacetanilide. Reacting with phosphorus it forms chlorobenzamide. Aniline, and many of its derivatives, readily reacts with oxygen. Most of the compounds formed by the reaction of aniline, or its derivatives, with oxygen and halides, tend to float upon the top of the arc extinguishing liquid, but are heavier than water. The same is true of the forms of such compounds in purifying tetrachloroethylene or trichloroethylene. The aniline and its products of reaction with oxygen and the halogens are substantially insoluble in halogen derivatives.

Certain other acid substances may be present in tetrachloroethylene and trichloroethylene, and the aniline which I employ as a preservative reacts with such acid substances to remove the same from the liquid. In the refining or purifying of halogen derivatives of the hydrocarbons with aniline, the precipitate is first formed and the liquid may then be filtered and distilled to remove the impurities. Distillation, however, is optional.

Instead of employing aniline as a preservative, that is, a neutralizer and acid remover for the dielectric bath, I may employ other materials which do not interfere with the dielectric properties and arc extinguishing characteristics of the same, when used in proper proportions, but which serve to react with the impurities that otherwise would cause breakdown of the liquid and attack of the metal parts.

As above mentioned, aniline dyes and products derived from aniline may be utilized. In addition, various nitrogen containing compounds of aromatic hydrocarbons, such, for example, as hydrazobenzene ( $C_6H_5NH-NH.C_6H_5$ ), azobenzene ( $C_6H_5N:NC_6H_5$ ) and azoxybenzene ( $C_12H_10N_2O$ ) as substitutes for aniline, may be used. The above compounds are all coal tar derivatives. Also some of the amino compounds of the aliphatic series, such as isopropylamine, acetamid, etc., may be employed as preservatives.

Whereas, in the above disclosure, I have referred to the dielectric bath, where the same has been discussed in detail, as consisting of one or more halogen derivatives of aliphatic hydrocarbons, I find that halogen derivatives of aromatic hydrocarbons may be employed for this service, that is, as an arc extinguishing liquid in circuit interrupters broadly and in liquid filled fuses specifically, and as a dielectric medium for electrical apparatus, such as high tension terminals, high tension cables, transformers and the like.

The preservatives which I have above disclosed as suitable for use in connection with the aliphatic halogen derivatives may be employed in preserving the aromatic halogen derivatives and/or purifying the same.

I therefore wish to include within the present invention the use of aliphatic and aromatic nitrogen containing compounds as preservatives and

purifiers of halogen derivatives of hydrocarbons of either the aromatic or aliphatic group. The aromatic compounds are generally called the ring compounds, being chiefly exemplified in benzene ( $C_6H_6$ ) and its derivatives. A number of compounds comprising halogen derivatives of aliphatic hydrocarbons, chiefly compounds of fluorine and chlorine, or both of them, have been developed in the chemical industry. Some of them are as follows.

| Compound     | Name                        | Degrees centi-grade boiling point | Nature  | 15 |
|--------------|-----------------------------|-----------------------------------|---------|----|
| $CHClF_2$    | Monochlorodifluoromethane   | -39.8                             | Gas.    |    |
| $CCl_2F_2$   | Dichlorodifluoromethane     | -29.8                             | Gas.    |    |
| $C_2F_4$     | Tetrafluoroethylene         | -80                               | Gas.    |    |
| $C_2F_6$     | Hexafluoroethane            |                                   | Gas.    |    |
| $C_2FC_2Cl$  | Monofluoropentachloroethane | 136.8                             | Solid.  | 20 |
| $C_2F_3Cl_2$ | Difluorotetrachloroethane   | 91                                | Solid.  |    |
| $C_2F_4Cl$   | Trifluorotrifluoroethane    | 48.5                              | Liquid. |    |
| $C_2F_5Cl$   | Monochloropentafluoroethane |                                   | Gas.    |    |
| $C_2F_6Cl$   | Dichlorotetrafluoroethane   |                                   | Gas.    | 25 |

The substances which are solids and liquids may be employed in fuses and for dielectric baths as herein described. I have also found that certain bromine derivatives of aliphatic hydrocarbons may be employed, some of the same being the following:

| Composition | Specific gravity | Degrees centi-grade boiling point | Degrees centi-grade freezing point | Nature  | 35 |
|-------------|------------------|-----------------------------------|------------------------------------|---------|----|
| $CBrCl_2$   | 1.959            | 172                               | -21                                | Liquid. |    |
| $CBr_2$     | 3.42             | 189.5                             | 48.4<br>B90.1                      | Solid.  | 40 |
| $CHBr_2$    | 2.890            | 147.5                             | 7.7                                | Liquid. |    |
| $CH_2Br_2$  | 2.48             | 97.8                              | -52.8                              | Liquid. |    |
| $C_2H_2Br$  | 2.964            | 161                               | .1                                 | Liquid. |    |
| $C_2BrCl_3$ | 2.304            | 172                               | 4.4                                | Liquid. |    |
| $C_2Br_2Cl$ |                  | 203                               | 34                                 | Solid.  |    |
| $C_2Br_3$   |                  | 226                               | 57                                 | Solid.  | 45 |
| $C_2HBr_3$  | 2.708            | 163                               |                                    | Liquid. |    |

Bromine derivatives are more easily oxidized by water and oxygen of the air than chlorine derivatives. Iodine derivatives may also be employed. In all of the above, the aliphatic and aromatic nitrogen containing compounds which I have above described, and a typical and preferred form of which is aniline, may be employed as purifiers and preservatives.

I am aware that paraffin hydrocarbon has been proposed as a preservative of tetrachloroethylene, but I wish to point to the fact that paraffin hydrocarbon is neutral with respect to acid impurities, and cannot combine with and remove the impurities.

Also, as a dielectric medium for extinguishing arcs, paraffin hydrocarbon is not desirable in that it is combustible, and adds to the energy liberated upon venting of the fuse to atmosphere. In other words, it tends to increase instead of decrease the flash and flame, as a large amount is required to preserve the liquid and prevent injury by the acid content.

The use of aniline or like nitrogen containing compounds, derivatives of hydrocarbons in conjunction with any of the above liquids or solids, has a further virtue that such preservative may combine with oxygen and still be available as a neutralizing medium for free acids or acid form-

ing compounds or radicals that may be found in or result from breakdown of the dielectric medium.

Aniline may also be called a reducing agent as it is easily oxidized, taking oxygen away from some other source. There are many reducing agents, I have found, which act much the same as aniline in this respect, which do not contain nitrogen in the molecule, such as pinene ( $C_{10}H_{16}$ ), 5 cymene ( $C_{10}H_{14}$ ), limonene ( $C_{10}H_{16}$ ) and ( $C_6H_5O_2$ ) hydroquinone, etc. They are not as efficient, however, as aniline, but I wish to claim the right to use these if and when the occasion should permit.

15 The aniline or equivalent purifier or preservative has, for my purposes, the valuable features with respect to the liquid, first, that such purifier will combine with free oxygen to prevent it attacking the dielectric; second, the purifier 20 will react with any acid contained in the dielectric or released by breakdown of the same; third, that such preservative does not substantially interfere with the properties and functions of the dielectric and, fourth, that the combination 25 products of such preservative with injurious impurities do not substantially injure the properties and functions of the dielectric.

The solid substitution products of a hydrocarbon containing a halogen may be employed in a 30 fuse of the type disclosed in the patent to Ringwald, No. 1,862,317, to which reference has previously been made.

The halogen derivatives of aromatic hydrocarbons may be employed with or without the 35 preservative herein disclosed for arc extinguishing and general dielectric purposes, within the scope of my invention.

I do not intend to be limited to the precise details herein shown and described, nor to the 40 specific compounds which I have referred to herein as classes suitable for the service herein referred to.

I claim:

1. In a device of the class described, the combination of a closed housing, a pair of metallic terminals between which an arc is adapted to be formed, and an arc extinguishing liquid in the housing, said liquid comprising a halogen derivative of a hydrocarbon and containing a small 45 amount of an aromatic nitrogen containing compound.

2. In an electrical device, a closed housing comprising two chambers, an electric fuse in said housing, one of said chambers being adapted to 50 contain an arc extinguishing liquid, the other of said chambers being adapted to contain air, an arc extinguishing liquid in said first chamber, said liquid being subject to reaction with the oxygen in the air chamber to yield an acid, and 55 a neutralizing agent in said liquid capable of preventing injury to said liquid by the oxygen and capable of reacting with the acid content of the arc extinguishing liquid.

3. In a device of the class described, the combination of a housing comprising an insulating sleeve having metallic ferrules forming terminals externally, a pair of metallic fuse terminals in said housing, a fuse electrically connecting said fuse terminals and adapted to be fused by excess 60 current flow through the device, metallic connections between said fuse terminals and said external terminals, an arc extinguishing material in said housing adapted to be acted upon by the heat of the arc to form a gaseous arc extinguishing medium, said material comprising a com-

and a protective compound in said housing, said protective compound inhibiting migration of said strongly active substance from said material to said metallic parts of the device.

4. In a device of the class described, the combination of a housing, a pair of fuse terminals, a fuse between said terminals, said fuse being adapted to be melted upon the flow of excess current through the device, an arc extinguishing material in said housing, said liquid comprising a halogen derivative of a hydrocarbon and containing a small amount of a compound having an alkaline reaction and easily combinable with oxygen.

5. In a device of the class described, the combination of a housing, a pair of fuse terminals, a fuse between said terminals, said fuse being adapted to be melted upon the flow of excess current through the device, an arc extinguishing material in said housing, said material comprising a halogen derivative of a hydrocarbon and containing a small amount of coal tar dye.

6. In a device of the class described, the combination of a housing, a pair of metallic terminals between which an arc is adapted to be formed, an arc extinguishing material disposed to be acted upon by the arc to evolve a gaseous arc extinguishing material, said arc extinguishing material being adversely affected by contact with the atmosphere and causing corrosion of the metallic parts, and a protective substance which does not substantially interfere with the arc extinguishing properties of said material for inhibiting the said corrosion.

7. In a device of the class described, the combination of a housing, a pair of metallic terminals between which an arc is adapted to be formed, an arc extinguishing material disposed to be acted upon by the arc to evolve a gaseous arc extinguishing material, said arc extinguishing material being adversely affected by contact with the atmosphere and causing corrosion of the metallic parts, and a protective substance cooperating with said material to protect the same from atmospheric influences, said substance being relatively small in proportion to the material and causing no substantial interference with the arc extinguishing properties of said material.

8. In a device of the class described, the combination of a closed housing, a pair of metallic terminals between which an arc is adapted to be formed in the housing, and a charge of arc extinguishing liquid in the housing comprising tetrachloroethylene containing a relatively small amount of aniline dissolved therein.

9. In a device of the class described, the combination of a closed housing, a pair of metallic terminals between which an arc is adapted to be formed in the housing, and a charge of arc extinguishing liquid in the housing comprising tetrachloroethylene containing a relatively small amount of a reagent capable of combining with and neutralizing any free acid in the housing.

10. In a device of the class described, the combination of a closed housing, a pair of metallic terminals between which an arc is adapted to be formed in the housing, and a charge of arc extinguishing liquid in the housing comprising tetrachloroethylene containing a relatively small amount of a basic compound capable of reacting with contained acid impurities.

11. In a device of the class described, the combination of a closed housing, a pair of metallic terminals between which an arc is adapted to be formed in the housing, and a charge of arc ex-

- 5 pound of a strongly active chemical substance, extinguishing liquid in the housing comprising tetrachloroethylene containing a small amount of a nitrogen containing derivative of a hydrocarbon.
12. In a device of the class described, the combination of a closed housing, a pair of metallic terminals between which an arc is adapted to be formed in the housing, and a charge of arc extinguishing liquid in the housing comprising a halogen derivative of a hydrocarbon containing a small amount of a nitrogen-containing derivative of a hydrocarbon. 5
13. In a device of the class described, the combination of a closed housing, a pair of metallic terminals between which an arc is adapted to be formed in the housing, and a charge of arc extinguishing liquid in the housing comprising a halogen derivative of hydrocarbon of the aromatic class containing a small amount of a nitrogen-containing derivative of a hydrocarbon. 10
14. In a device of the class described, the combination of a closed housing, a pair of metallic terminals between which an arc is adapted to be formed in the housing, and a charge of arc extinguishing liquid in the housing comprising a halogen derivative of a hydrocarbon containing a relatively small amount of a compound capable of combining with the oxygen of the air, said amount being not substantially more than one-tenth of one per cent by weight. 15
15. In a device of the class described, the combination of a closed housing, a pair of metallic terminals between which an arc is adapted to be formed in the housing, and a charge of arc extinguishing liquid in the housing comprising a halogen derivative of an aliphatic hydrocarbon containing a relatively small amount of a nitrogen-containing derivative of a hydrocarbon. 20
16. In a device of the class described, the combination of a closed housing, a pair of metallic terminals between which an arc is adapted to be formed in the housing, and a charge of arc extinguishing liquid in the housing comprising tetrachloroethylene, trichloroethylene and aniline. 25
17. In a device of the class described, the combination of a closed housing, a pair of metallic terminals between which an arc is adapted to be formed in the housing, and a charge of arc extinguishing liquid in the housing comprising trichloroethylene in mixture with tetrachloroethylene in the proportions of substantially 10% to 6% of the former and 90% to 94% of the latter containing a relatively small amount of a dissolved preservative which is oxidizable by contact with air. 30
18. In a device of the class described, the combination of a closed housing, a pair of metallic terminals between which an arc is adapted to be formed in the housing, and a charge of arc extinguishing liquid in the housing comprising hexachloroethane and tetrachloroethylene, said liquid containing a relatively small amount of a preservative which is oxidizable by contact with atmospheric oxygen at room temperatures. 35
19. In a device of the class described, the combination of a closed housing, a pair of metallic terminals between which an arc is adapted to be formed in the housing, and a charge of arc extinguishing liquid in the housing comprising a halogen derivative of hydrocarbon and a small amount of a preservative capable of combining with acid impurities to neutralize the same, and capable of combining with free oxygen upon exposure thereto, without substantial in- 40
- jury to the properties of said composition of matter for arc extinguishing purposes, said amount being not substantially more than one-tenth of one per cent by weight. 45
20. In a device of the class described, the combination of a housing, a pair of metallic terminals between which an arc is adapted to be formed in the housing, a charge of arc extinguishing material in the housing in position to be acted upon by the heat of the arc to evolve a gaseous arc extinguishing medium, said material comprising a halogen derivative of a hydrocarbon with a small amount of basic material, the compounds formed by said basic material and the impurities contained in said first material being substantially insoluble. 50
21. In a device of the class described, the combination of a housing, a pair of metallic terminals between which an arc is adapted to be formed, a charge of arc extinguishing material in the housing in position to be acted upon by the heat of the arc to evolve a gaseous arc extinguishing medium, said material comprising a halogen derivative of a hydrocarbon and a small amount of a reducing agent. 55
22. In a circuit interrupting device having a housing pervious to light, metallic conducting parts, a charge of liquid arc extinguishing material in the housing in contact with said metallic parts, said liquid under the action of light or heat and in contact with air or moisture causing corrosion of said metallic parts, and an inhibitor present in small amounts as herein described for preventing corrosion of said metallic parts when said liquid is subjected to the aforesaid influences. 60
23. In a circuit interrupting device of the class described, comprising a closed chamber containing metallic conducting parts, a charge of liquid comprising a halogen derivative of a hydrocarbon, and a body of inert gas contained in said chamber above said liquid. 65
24. A liquid charged fuse having a charge of liquid comprising a halogen derivative of a hydrocarbon and a body of nitrogen gas contained in the fuse above the liquid. 70
25. A fuse having a closed housing, metallic parts including a fusible link in the housing, an arc extinguishing material in the house in close proximity to said metallic parts, and a charge of an inert gas in the housing into which gas metallic vapor produced by blowing of the link is projected. 75
26. In a circuit interrupter having a housing pervious to light, an arc extinguishing liquid comprising a halogen derivative of a hydrocarbon and a coal tar dye permeating the same, said dye being capable of absorbing a portion of the spectrum of the sunlight falling upon the liquid to avoid deterioration of the liquid. 80
27. In a liquid containing fuse having a housing pervious to light, an arc extinguishing liquid comprising a halogen derivative of a hydrocarbon and a coal tar dye permeating the same, said dye being capable of absorbing a portion of the spectrum of sunlight falling upon the liquid and being further capable of combining with free oxygen in contact with the liquid and capable of neutralizing decomposition products of the liquid to render said products non-corrosive upon metallic parts of the fuse. 85
28. In a device of the class described, a housing containing metallic conducting parts, a charge of normally neutral liquid dielectric in

contact with the metallic parts in the housing, said liquid being subject to influences which cause it to develop corrosive properties, and a nitrogen containing compound present in small amounts for preventing the development of said corrosive properties.

29. An arc extinguishing liquid for circuit interrupters, said liquid comprising tetrachloroethylene, trichloroethylene and aniline.

10 30. As an arc extinguishing liquid for use in circuit interrupters, trichloroethylene in mixture with tetrachloroethylene in the proportions of substantially 10% to 6% of the former and 90% to 94% of the latter containing a relatively small 15 amount of a dissolved preservative which is oxidizable by contact with air.

31. An arc extinguishing liquid for use in circuit interrupters, a liquid comprising hexachloroethane and tetrachloroethylene, said liquid containing a relatively small amount of a preservative which is oxidizable by contact with atmospheric oxygen at room temperatures.

32. As an arc extinguishing liquid for use in an electric fuse, a halogen derivative of hydrocarbon and a small amount of a preservative capable of combining with acid impurities to neutralize the same, and capable of combining with free oxygen upon exposure thereto, without substantial impairment of the properties of said liquid for arc extinguishing purposes, said amount being not substantially more than one-tenth of one per cent by weight.

33. In an electrical device, a closed housing comprising two chambers, circuit interrupting means in said housing, one of said chambers containing an arc extinguishing material, the other of said chambers containing a gas, and a neutralizing agent in the arc extinguishing material capable of preventing the formation of injurious 40 compounds by contact of the gas therewith.

34. In a circuit interrupter, a closed housing, metallic parts including separable terminals between which an arc is adapted to be drawn, an arc extinguishing material in the housing in effective proximity to said terminals, and a charge of an inert gas in the housing, the products of the arc being discharged into said gas.

35. In a circuit interrupter, a closed housing including a cooling chamber having an extensive surface and containing a charge of an inert gas, separable terminals between which an arc is adapted to be established in the housing disposed adjacent said chamber, and an arc extinguishing material in the housing in close proximity to said separable terminals and adapted to be acted upon by the arc between them, the products of the arc being discharged into said cooling chamber.

36. In a circuit interrupting device having a housing pervious to light, in combination, metallic conducting parts, a charge of liquid arc extinguishing material having a halogen content of over 75% by weight in said housing in contact with said metallic parts, said liquid under action of light or heat and in contact with air or moisture causing corrosion of said metallic parts, and an inhibitor present in small amounts as here-

in described for preventing corrosion of said metallic parts when said liquid is subjected to the aforesaid influences.

37. In a circuit interrupting device, in combination, metallic conducting parts, a charge of liquid arc extinguishing material having a halogen content of over 75% by weight in contact with said metallic parts, said liquid being disposed to cause corrosion of said parts on change in temperature thereof in contact with air or moisture, and an inhibitor present in small amounts as herein described for preventing corrosion of said metallic parts when said liquid is subjected to said influences.

38. In a circuit interrupting device having metallic conducting members, in combination, a charge of liquid arc extinguishing material having a halogen content of over 75% by weight in contact with said conducting members, said liquid in the presence of air or moisture being disposed to cause corrosion of said conducting members, and an inhibitor present in small amounts as herein described for preventing corrosion of said conducting members on the occurrence of said conditions.

39. In a current conducting device adapted to remain in service undisturbed for extended periods of time, the combination of a casing sealed to exclude entrance of air and moisture, a metallic electrical conductor in said casing, said electrical conductor having circuit completing connections outside the casing, a halogenated hydrocarbon forming a dielectric filling for said casing for insulating said conductor and for extinguishing any electric arc that may be formed within said casing, and a corrosion inhibitor in said casing dispersed in said dielectric filling sufficient to combine with chemical impurities which may be formed from confined air and moisture but insufficient to produce any substantial impairment of the dielectric or arc extinguishing properties of the dielectric filling.

40. The combination of claim 39 wherein the corrosion inhibitor comprises aniline.

41. The combination of claim 39 wherein the inhibitor is a nitrogen containing derivative of a hydrocarbon.

42. The combination of claim 39 wherein the dielectric filling is a liquid comprising tetrachloroethylene and the inhibitor is an oxidizable hydrocarbon substitution product capable of combining with chlorine compounds.

43. The combination of claim 39 wherein the dielectric filling comprises trichloroethylene substantially 10% to 6% and tetrachloroethylene substantially 90% to 94% and the inhibitor is an amino compound of hydrocarbon.

44. The combination of claim 39 wherein the inhibitor is an oxidizable organic compound.

45. The combination of claim 39 wherein the dielectric filling is a liquid comprising trichloroethylene and the inhibitor is an oxidizable hydrocarbon substitution product capable of combining with chlorine compounds.

GEORGE F. McMAHON. 65

CERTIFICATE OF CORRECTION.

Patent No. 2,077,429.

April 20, 1937

GEORGE F. McMAHON.

It is hereby certified that error appears in the printed specification of the above numbered patent requiring correction as follows: Page 6, first column line 75, claim 3, after the syllable "com-" add the syllable words and comma pound of a strongly active chemical substance; second column, line 40, claim 7, for "extitnguishing" read extinguishing; and page first column, line 1, claim 11, strike out the words and comma "pound of strongly active chemical substance,"; and that the said Letters Patent should be read with these corrections therein that the same may conform to the record of the case in the Patent Office.

Signed and sealed this 13th day of July, A. D. 1937.

Henry Van Arsdale

(Seal)

Acting Commissioner of Patents.